

# UNITED STATES PATENT OFFICE.

ALEC GAVAN INRIG, OF TOTTENHAM, ENGLAND, ASSIGNOR OF THREE-FOURTHS TO HERBERT EDWARD MCKRELL, OF WESTMINSTER, ENGLAND.

## TREATMENT OF WASTE LEATHER, RAWHIDES OR SKINS, HOOFS, HORNS, OR BONES OF ANIMALS.

No. 892,840.

Specification of Letters Patent.

Patented July 7, 1908.

Application filed October 5, 1906. Serial No. 337,646.

*To all whom it may concern:*

Be it known that I, ALEC GAVAN INRIG, consulting engineer, a subject of the King of Great Britain, residing at 83 Bruce Grove, 5 Tottenham, in the county of Middlesex, England, have invented certain new and useful Improvements in or Relating to the Treatment of Waste Leather, Rawhides or Skins, Hoofs, Horns, or Bones of Animals, of 10 which the following is a specification.

This invention relates to the treatment of waste leather raw hides or skins hoofs horns or bones of animals and has for its object the production from said material or materials 15 and certain chemicals of a new or improved substance or compound which may be applied to any desired purposes for example it may be utilized (as a substitute for india-rubber or gutta-percha) for many of the purposes 20 for which india-rubber or gutta-percha is applicable for instance this new or improved substance or compound may be used in a squirting machine for covering and insulating electric wires and cables; it may be 25 rolled into sheets (with or without canvas or the like) and cut into strips or rolls of tape for lapping electric cables or it may be molded and vulcanized for any desired purpose *e. g.* for electric accumulator cells, or it 30 may be made so as to serve as a substitute for leather, vulcanite, etc., etc.

According to this invention the material or materials (waste leather, raw hides or skins, hoofs, horns, or bones of animals—or 35 any mixture thereof) are placed in a suitable vessel and boiled for an hour (or more or less as desired) in water to which has been added a small quantity of caustic soda or other suitable alkali; the quantity of alkali used 40 being determined by the quality of the material to be treated and is usually from about 3% to 10% or more or less as required. After boiling as aforesaid the mass is allowed to cool; and for this purpose it may or 45 may not be removed to another vessel, and in the case of waste leather raw hides or skins it is reduced to a pulp by the aforesaid means of heat and an alkali which is a good solvent of leather. The action of the alkali 50 is arrested before the mass has been reduced to a glue; and the mass is then treated with dilute sulfuric acid of suitable density—say 1.200 density or more or less as desired; in this treatment the relative proportion of 55 acid used will be determined by the quantity

of alkali that has been applied in the boiling. About one gallon dilute acid for every 1% of alkali used in the boiling process gives a good result. Next—when treating waste leather raw hides or skins—a gentle heat is applied 60 to the mass (by means of a steam jet or otherwise and as this mass of waste leather raw hides or skins (all of which for the sake of brevity will hereinafter be referred to as “waste leather”) warms up a new material 65 or substance is formed which separates itself from the water and rises to the surface after the manner of froth and this material is then skimmed off (or the water may be drawn off and the material removed) and utilized in 70 any of the following manners:—For example it may now be thoroughly dried and (with or without further treatment) it may under heat be rolled pressed or molded into any suitable form shape or article desired for instance it may be pressed in hot dies into sheets of any desired thickness for electrical or other purposes; or for certain purposes, such as for forming heels for boots and 75 shoes, parquet blocks, fireproof floorings, partitions, and ceilings etc. the following mixture may be employed:—10% or thereabout of waste leather treated and prepared as aforesaid may be mixed with 90% or thereabout of sawdust. This mixture is 80 then damped with a solution made up of 1% of stannate of soda and 2% of hide glue. This material in a cold state is thoroughly 85 mixed and it may then be heated and laid down hot on the wood iron concrete or other 90 surface to be coated or covered, and leveled down with hot irons; or this mixture in the cold state may be placed in any suitable mold or press and pressed or molded under heat (*e. g.* in hot dies) and so formed into 95 boards or parquet blocks heels for boots and shoes etc. Or before treating the waste leather in the aforesaid manner, such waste leather may have mixed therewith any suitable proportion of other waste materials 100 such as rags of any description, waste paper, or straw; such mixture of waste leather and such waste material being boiled together in the alkali, and then treated with an acid as hereinbefore described with reference to the 105 waste leather alone; and after leaving the acid tank there is added to this mixture of materials 1% of stannate of soda and 2% of hide glue; and this mixture of materials (when cold) is then thoroughly mixed and 110

may then be utilized as above described with reference to the mixture of leather and sawdust. Or according to a further part of the present invention the new substance or material thus produced from leather waste 5 may be further treated and mixed with bitumen as hereinafter described.

In the case of the leather waste, after same has been subjected to the foregoing 10 treatment and the new material or substance obtained as aforesaid (*i. e.* after the alkali and acid treatment) such material as it rises to the surface is skimmed off (or the water may be drawn off) and the material removed 15 to a suitable vessel which may advantageously be an ordinary steam jacketed masticator or other suitable vessel wherein it is mixed with an equal or other suitable quantity of Trinidad bitumen or the like advantageously bitumen specially prepared as hereinafter described.

The bitumen used is advantageously that—or of the character of that—known as Trinidad bitumen; a quantity of which is 20 placed in a suitable boiler and raised to a temperature of 260° to 300° F.; and to this bitumen there is then added 20% (or other suitable proportion) of petroleum residuum or animal fat, 15% (or other suitable proportion) of sulfur, 10% (or other suitable proportion) of glutinous material such as horn hoof or bone meal, or glue, etc. This mixture is stirred or agitated for one hour or thereabout and kept at about 300° F. for 25 another hour or thereabout, and is then ready to be mixed with the aforesaid waste leather product in the steam jacketed masticator or other suitable mixing vessel.

After thoroughly mixing this waste leather 30 product and prepared bitumen as aforesaid in the masticator for about 45 minutes (or more or less) at a temperature of about 240° F. the material may be rolled into sheets and cut up for the squiring machine or spread 35 on canvas and cut up to form an insulating tape, or utilized in any other desired manner.

Other suitable proportions of the waste leather product and the prepared bitumen 40 may be used if desired for example 75% of the waste leather product and 25% prepared bitumen may be employed the resulting mixture being suitable for molding into accumulator boxes and other electric insulating purposes, or may be employed for any other 45 desired purposes.

Referring now to the case of horns hoofs 50 and bones—after same have been subjected to the alkali and acid treatment—the resulting mass (which tends to settle in the vessel and therefore does not rise in the form of a froth as in the case of the waste leather raw 55 hides or skins) is now passed through a pair of rollers having different peripheral speeds (or through more than one such pair of differential rollers if desired) and dried; and

the resulting dry powder may be utilized (without further treatment) by pressing or molding into shape under heat. Or according to a further part of the present invention the hoofs horns or bones thus prepared may 70 then be treated or mixed with bitumen (prepared as aforesaid) as follows:—The horns, hoofs, or bones, (either any one thereof alone or any mixture thereof) are treated with caustic soda under heat, and then cooled and 75 treated with sulfuric acid to neutralize the alkali as hereinbefore described, and the mass thus treated is then reduced to a fine powder by any suitable means for example by repeatedly passing it through rollers having 80 different peripheral speeds and drying it.

This powder is then mixed with about 30% of Trinidad bitumen prepared as aforesaid or the like and is then thoroughly dried and 85 may now be utilized in any desired manner *e. g.* it may be pressed into sheets rods or tubes by means of hot dies, under a hydraulic press and the resulting product is a black or dark substance resembling ebony possessing 90 very high electrical resisting properties and this mixture of horns hoofs or bones and prepared Trinidad bitumen is absolutely non-hygroscopic.

This invention is not confined to the exact figures and proportions as hereinbefore described.

In some cases as for instance with pieces of hard leather such as old leather soles and cuttings from sole leather or from hydraulic pressed leather it is found advantageous to 100 first immerse such hard pieces of leather in a solution of water and lime (*i. e.* milk of lime) in which it is heated and to which is added the alkali as aforesaid; this addition of lime facilitating the softening of the leather and 105 reducing the length of time during which it is necessary to boil it.

What I claim is:—

1. The herein described process of producing from waste leather raw hides and skins, 110 hoofs, horns or bones a new substance or compound which consists in treating waste leather etc. first with an alkali under heat arresting the action thereof before a glue is formed and then after cooling the mass treating 115 the latter with a dilute acid, drying the mass, and finally molding it or subjecting it to pressure.

2. Process of producing from waste leather raw hides or skins and chemicals a new and 120 useful substance or compound which consists in reducing such waste leather raw hides or skins to a pulp by means of heat and an alkali, cooling the mass and arresting the action of the alkali before glue is formed 125 treating the mass with an acid and then again applying heat to the mass and thereby converting the aforesaid materials into a new substance or compound which may then be utilized in any desired manner.

3. The herein described process of producing material in suitable form for heels for boots and shoes fireproof flooring or partitions or the like or other purposes, which 5 consists in treating waste materials such as leather, raw hides, skins, hoofs, horns or bones, first with alkali under heat, arresting the action thereof before a glue is formed, then after cooling the mass, treating the 10 same with dilute acid, then mixing sawdust with the new substance just formed damping this mixture with a solution of stannate of soda and hide glue the mass being ground and thoroughly mixed and either applied hot 15 to the surface to be coated therewith or molded or pressed under heat into any suitable form substantially as set forth.

4. Process of producing from waste leather raw hides or skins hoofs horns or bones of 20 animals and chemicals a new and useful substance which consists in treating waste leather raw hides or skins hoofs horns or bones with alkali under heat, arresting the action before a glue is formed cooling the mass and treating the same with a dilute acid and mixing the resultant product with bitumen substantially as set forth.

5. Process of producing from waste leather raw hides or skins hoofs horns or bones of

30 animals and chemicals a new and useful substance which consists in treating waste leather raw hides or skins hoofs horns or bones with alkali under heat, cooling the mass and arresting the action of the alkali by treating the mass with an acid and mixing 35 the resulting product with specially prepared Trinidad bitumen substantially as set forth.

6. The herein described process of producing a material in a suitable form, for heels of boots and like articles which consists in treating waste leather, raw hides, skins, hoofs, horns or bones, first with an alkali under heat, arresting the action thereof before a glue is formed, then cooling the mass treating the latter with dilute acid mixing the 40 same with sawdust damping this mixture with a solution of stannate of soda and hide glue, grinding the mass and thoroughly mixing the same with prepared Trinidad bitumen and finally molding the resultant product 45 into suitable forms, substantially as set forth.

In witness whereof I have hereunto set my hand in presence of two witnesses.

ALEC GAVAN INRIG.

Witnesses:

FREDK. L. RAND,  
A. NUTTING.